

## UNITED STATES PATENT OFFICE.

FREDERICK M. BECKET, OF NEW YORK, N. Y.

## ANODE FOR CHROMIUM PLATING.

No Drawing.

Application filed October 14, 1926. Serial No. 141,678.

This invention relates to the art of electroplating with metallic chromium, and comprises a soluble, chromium-containing cast anode for use in that operation.

5 Heretofore such anodes have commonly been made of cast chromium of the highest purity which was commercially available, hereafter for brevity designated "pure chromium".

10 Anodes of pure cast chromium present a number of undesirable properties. Pure chromium is quite viscous even when heated to a temperature well above its melting point, so that anodes can be cast from it only 15 in the simplest shapes. Such anodes are porous in varying degree, so that their rate of solution in the chromic acid electrolyte is irregular and impossible to predetermine. Furthermore, the crystal structure is such as 20 to affect most unfavorably the manner in which the anodes dissolve: instead of dissolving smoothly and regularly they tend to disintegrate, pieces of various sizes spalling or sloughing off and collecting at the bottom 25 of the electrolytic cell, this involving not only an increase in anode consumption but interfering with the operation of the cell.

These and perhaps other deficiencies of 30 cast chromium anodes have been heretofore recognized, and have been summarized somewhat inaccurately by characterizing such anodes as "brittle". It has been proposed to lessen this "brittleness" by addition of 35 lead, cobalt, iron or nickel; and while some of these additions in some proportions may diminish the so-called brittleness of the anode, they have the disadvantage that eventually they either foul the bath or have an 40 undesirable effect upon the quality of the deposit.

According to the present invention the 45 defects mentioned above are overcome, and further advantages are secured, by alloying the chromium with certain proportions of silicon, the amount of silicon varying with the objective to be attained, as explained below.

50 Silicon performs three distinct functions: 1. In the smaller percentages it increases the fluidity of the molten metal, facilitates the casting, and improves the grain of the cast article. These effects are already noticeable with silicon additions as low as 0.25 percent; but in case these are the chief ob-

jectives I prefer to introduce one to two percent of silicon, as already stated.

2. It is characteristic of metallic chromium anodes, used in a chromic acid electrolyte, that they tend to dissolve more rapidly than 60 corresponds to the deposition of metal at the cathode, with the result that the concentration of the bath tends to increase progressively, and corresponding irregularities are introduced into the operation. This difficulty has been overcome in the past by the simultaneous employment of soluble (chromium) and insoluble (lead) anodes, as disclosed in U. S. Patent 1,544,451 to Hambuechen. I have discovered that silicon, 65 alloyed with the chromium in sufficient proportions, reduces the solubility of the chromium in the electrolyte, such as aqueous solutions of chromic acid. The solubility of the chromium diminishes progressively as 70 the percentage of silicon is increased, until at about 40 percent silicon and upward, the balance almost all chromium, the alloy functions practically like an insoluble anode. Accordingly it is possible by properly adjusting the silicon content so to control the 75 rate of solution of chromium as to obtain the desired balance between the amount of metal dissolving at the anode and the amount deposited at the cathode, whereby the electrolyte remains within the limits of concentration suitable for efficient plating. It is of course impossible to specify a definite silicon content which will accomplish this result in 80 every case, because the cathode efficiency 85 varies considerably with the type of electrolyte used, its concentration and temperature, the current density, and other factors; but for use in baths consisting predominantly 85 of chromic acid in aqueous solution, I find 90 that the optimum percentages of silicon lie 95 between 10 and 35 percent; and in most cases between 20 and 30 percent.

3. Silicon in sufficiently high proportion 100 is capable of practically excluding carbon from the chromium-silicon alloy. For example a chromium-silicon alloy containing about 40 percent of silicon, or upward, prepared by carbon reduction in an electric furnace of a charge of chromic oxide and silica, will contain only a fraction of one percent of carbon: and this practically carbon-free chromium-silicon alloy may be refurnaced with chromium oxide to oxidize out 105 any desired proportion of the silicon. In 110

this way I am enabled to prepare alloys containing not more than 0.5 percent of carbon, the balance substantially all chromium and silicon, the silicon in any desired proportion. Such alloys are regarded, for the purposes of this invention, as substantially carbon-free.

Having regard to all of the above-described functions of silicon, it will be understood that my present invention comprises an anode of cast chromium metal containing silicon in proportion between about 0.25 percent and 35.0 percent, according to the particular objectives to be attained, the alloy being substantially carbon-free or containing carbon not in excess of 0.5 percent. Cast chromium anodes containing carbon 0.5 to

7.0 percent, and with or without silicon, are claimed in my copending application, Ser. No. 141,667, filed October 14, 1926.

20

I claim:

1. In combination, an electrolyte consisting predominantly of an aqueous solution of chromic acid, and a substantially carbon-free anode comprising chromium and about 0.25 to 35 percent of silicon.

2. In combination, an electrolyte adapted to the electrodeposition of chromium, and a substantially carbon-free anode containing 0.25% to 35% of silicon, the balance of said anode being principally chromium.

In testimony whereof, I affix my signature.

FREDERICK M. BECKET.